

April 19, 1932.

R. C. STANLEY

1,854,234

PROCESS FOR RECOVERY OF NICKEL

Filed Aug. 17, 1929



INVENTOR  
Robert C. Stanley  
BY  
Byrnes, Stebbins & Parmentee  
ATTORNEYS

## UNITED STATES PATENT OFFICE

ROBERT C. STANLEY, OF DONGAN HILLS, NEW YORK, ASSIGNOR TO THE INTERNATIONAL NICKEL COMPANY, INC., OF NEW YORK, N. Y., A CORPORATION OF DELAWARE

## PROCESS FOR RECOVERY OF NICKEL

Application filed August 17, 1929. Serial No. 386,580.

This invention relates to an improved process for more readily and efficiently obtaining nickel and copper from the ores and to obtain these products directly and in readily 5 marketable forms.

More in particular the invention pertains to a novel process wherein the sequence of operations is carried out in the so-called dry way thereby eliminating the undesirable use and 10 handling of any material quantities of liquids.

It is an object of the present invention to provide an improved process for the recovery of metals from their ores by a sequence of 15 associated metallurgical steps, all of which are carried out without the aid of any material amount of water, or in what is known as the dry way.

It is a further object of this invention to 20 provide such an improved process for the recovery of nickel in a dry way from its ores, together with a direct recovery of copper as blister copper without resorting to the formation of aqueous solutions of copper salts.

Yet another object of this invention is the 25 preliminary treatment, in the dry way, of nickel-bearing materials to obtain an impure metallic nickel, and blister copper as a by-product, and the subsequent treatment of the 30 impure nickel to obtain a pure nickel.

This invention provides an improved process that is highly economical and low in cost and in which, by the association in a novel 35 manner of the steps set forth, a distinct increase in the efficiency of the complete process is obtained.

Another object of this invention is the provision of a process in which the percentages of nickel and copper in the mattes may vary 40 a considerable amount over what has heretofore been considered as desirable limits, and still obtain very satisfactory and economical results in the production of the copper and nickel.

The foregoing and other objects and advantages of the present invention will be set forth more in detail in the following specification, reference being had to the accompanying flow sheet as illustrating the preferred sequence of steps in the operation of

the improved process, but since other processes may be devised to accomplish the desirable results of the present invention, it is not intended to be limited to the steps herein shown except as such limitations are clearly imposed by the appended claims. 55

It is well known that there are several processes by which nickel and copper are produced from nickel-bearing materials. It is also well known that some of these processes 60 are carried out with greater efficiency than others.

One of the principal processes employed in separating nickel from copper-nickel ores and mattes today is that known as the Mond process. In this process the copper-nickel matte is crushed, ground and roasted to oxide and by a complicated leaching process, a part of the copper is removed from the mixed 65 oxides, leaving a nickel-oxide residue containing substantial amounts of copper and iron as impurities; following this, the residue is treated by the so called carbonyl process to further refine the nickel and separate the balance of the copper and other impurities. It 70 is an undesirable feature of the Mond process as at present practiced that a major part of the operation is carried out in the wet way involving high costs and producing copper in the form of copper sulphate, in considerable 75 quantities which is not a readily salable product. It is possible, of course, to recover metallic copper from this copper sulphate but only at a rather considerable cost, and at a large loss of efficiency. It will be seen from the description below of the process herein 80

that it obviates the principal defects of the Mond process and very materially reduces the amount of copper sulphate produced. When there is a relatively small amount of this copper sulphate it may be sometimes sold at a satisfactory price which compensates for the manufacture and handling thereof. 85

Another principal process for producing nickel is that known as the Stanley process, 90 which involves as a final operation the electrolytic refining of the nickel, and which is described in U. S. Patent No. 1,351,877. The nickel produced by this process is in the form primarily of cathode sheets, which, although 100

quite suitable for many types of remelting operations, do not constitute the preferable form for some operations, particularly those conducted on a small scale, such as crucible melting, etc. In order to convert nickel cathode sheets into shot form suitable for small scale melting operations, it is necessary that it be remelted, of course at an additional cost. The nickel produced by the Stanley process 10 has a small amount of cobalt therein. This cobalt content is not serious for most uses, but when the nickel is free of cobalt it may be more advantageous for some new and additional uses. It will be seen from the description of the process that it yields a product having certain material advantages, both in quality and in form, over those produced by the electrolytic processes above mentioned.

Another process, commonly known as the 20 Orford process, includes the smelting of copper-nickel ores and matte with sodium or alkaline sulphides to produce a partial separation of the copper and of the nickel sulphide, following which the nickel sulphide is subjected to chloridizing, roasting and leaching to remove the copper present as an impurity in the nickel sulphide in soluble form. The impure nickel oxide residue remaining after the leaching operation is reduced and melted 30 to metallic nickel. This process produces satisfactory metallic nickel, but it is necessary to resort to the wet process of separating part of the copper from the nickel, which involves increased costs, and in addition it is 35 not possible by it to recover all of the gold, silver, platinum, cobalt, copper, and other metals which may be present, and the nickel produced is not completely free from cobalt which may be present in small amounts.

40 The practical advantages of the improved invention herein have been noted above, but the novel process proceeding in the dry way gives readily marketable nickel and metallic blister copper and has given greater efficiency and economy of operation and greater quantity yield without requiring the close attention that has heretofore been necessary. The more important advantages may be summarized as follows: Low cost of production; improved efficiency; substantially complete recovery of precious metals including platinum, palladium, gold, silver and the like; the products are produced in advantageous form; and gives improved quality 55 and purity and particular absence of cobalt.

Referring now to the flow sheet, the improved process will be defined step by step.

A suitable nickel-bearing matte or other nickel-bearing material is subjected to a first 60 smelting, such as by treating with alkaline sulphides. The product of such smelting is permitted to settle so that the copper sulphide "tops" and the nickel sulphide "bottoms" may readily separate. It will be understood that in the copper sulphide tops

there will be a small percentage of nickel sulphide, and that in the nickel sulphide bottoms there will be a small percentage of copper sulphide. Also, this separation may be by either of two methods: The first allows the tops and bottoms to become solidified and later separated by breaking them apart. The second method is to produce and maintain a heated settler in which the products of the first and/or second smeltings 75 are introduced and then allowed to settle and are then drawn off separately in molten condition.

The copper sulphide tops pass to suitable converters where they are blown to metallic 80 blister copper. This production of the copper is an improvement over the Mond process in that the copper so produced requires only the customary electrolytic refining treatment in order to put it into metallic marketable 85 form, and is not produced in the form of crystallized copper sulphate or in an aqueous solution of copper sulphate.

There is a further economy resulting from the elimination of the copper leaching treatment in the Mond process as ordinarily practiced. In the operation of leaching the copper oxide, substantial amounts of nickel oxide are also dissolved in solution and are only recoverable in the form of crystallized 95 nickel sulphate. This results in a net loss of metallic nickel from the process and in the production of relatively less valuable product in its place.

The nickel sulphite bottoms are usually 100 submitted to another smelting step, and the products thereof are permitted to separate as described above. The copper sulphide tops of the second smelting are usually 105 passed back to the first smelting in order to obtain a purer copper and to be able to introduce more sulphides into the first smelting step, and also to thereby accomplish another economy whenever the sodium sulphide flux is first added to the process by being introduced into the second smelting step. 110

The nickel sulphide bottoms of the first or second smelting are crushed and ground, and leached, if desired. The leaching which is usually a water leaching, acts to remove only the sodium or alkali sulphides whenever it is desired to remove these sulphides. The leaching may also remove other soluble impurities. The small amount of water employed during the leaching process is not sufficient to warrant the use of the term liquid as generally used in processes of producing nickel, for the reason that none of the metal goes into solution from which it must later be recovered. 115

The thus produced nickel sulphide or compound leached or not is roasted to yield impure nickel oxide, the sulphur dioxide being liberated. The impure nickel oxide thus formed is then subjected at temperatures 120

from 200° C. to 600° C. to the action of a reducing gas, such as water gas or producer gas, preferably in a multiple hearth type furnace, hereinafter called a reducer, and is thereby reduced to an impure metallic nickel possibly containing small amounts of other metals such as gold, silver, copper, cobalt, and the metals of the platinum group and iron. In order to improve the reducing efficiency of this gas and to put the resulting reduced oxide into the best form and condition for later volatilization operations, this reducing gas may have added to it in the proper amounts, certain other reagents including water vapor and others.

The nickel or nickel-bearing materials coming from the reducer furnaces are then passed to similar furnaces, hereinafter called volatilizers, where they are continuously subjected to the action of carbon monoxide gas, preferably at a temperature approximating 80°-100° C. There may be added to this carbon monoxide gas for the volatilizers certain other reagents such as SO<sub>2</sub> or water vapor which act to hasten the volatilization rate of nickel. The volatilizers are of the multiple hearth type furnace, which permits the solid matter therein to be continuously subjected to a gaseous atmosphere. At the indicated temperature the carbon monoxide unites with the nickel to form the volatile compound—nickel carbonyl (Ni(Co)<sub>4</sub>), which passes to decomposers where the carbonyl is readily decomposed. The decomposers are usually vertical chambers in which carbon monoxide gas carrying nickel carbonyl is brought into intimate contact with metallic nickel at a temperature of from 125° C. to 250° C., at which temperature decomposition of the carbonyl occurs, resulting in deposition of metallic nickel. This nickel is deposited on small nickel pellets or upon any surface which is to be coated.

The depositing of the nickel on the small nickel pellets and the removal of the larger pellets is so well known in the art that further explanation thereof is not thought to be needed. The nickel pellets or nickel shot, as they may sometimes be called, are readily marketed and used in the preparation of different types of alloys requiring nickel as one of the constituents.

The carbon monoxide set free in the decomposition step is returned to an earlier stage of the process and permits further economies by virtue of its high efficiency and ease of manipulation.

The residues from the volatilizers may be subjected to any special treatments to remove the remainder of the copper, the gold, silver, cobalt, the metals of the platinum group, iron, etc.

It is to be noted that although the process herein effects many economies in the production of nickel and copper, and gives many ad-

vantages pertaining to the production of these materials, it is, however, particularly pointed out that the recovery of the precious metals also is accomplished with an increased efficiency and economies over other processes. By this improved process greater concentrations of precious metal values are accomplished with less effort or involved procedures to effect concentrations than are necessary in the refining of precious metals in general. This applies to the gold, silver, platinum, palladium and other precious metals which are normal constituents of nickel-bearing materials.

Another feature presented by this improved process is the fact that through the use of roasted nickel sulphide bottoms an unnecessary production of copper nickel sulphate salt, common to the older Mond process, is eliminated to a very large degree.

It will be appreciated that by the novel combination of steps comprehended in the process of the present invention a new and improved result is obtained in a much more satisfactory and economical manner.

The improved process of the present invention, among other things, permits the production of copper in metallic form, whereas, at the same time, it utilizes the highly desirable feature of the carbonyl separation method. In consequence the efficiency of this improved complete process is increased and the cost materially reduced. Further, the efficiency of the volatilization step of the carbonyl separation is actually increased when using the leached, roasted and reduced product of the alkaline sulphide smelting process.

In fact, it has been found that nickel materials produced by roasting sulphides as produced in the alkaline smelting process are more readily volatilized through the action of carbon monoxide than materials produced by roasting copper nickel sulphides with subsequent acid copper leaching to remove copper preliminary to the volatilization treatment.

It will now be appreciated that there has been provided an improved process for the recovery of metallic nickel from copper-nickel mattes of varying compositions which process permits the recovery of metallic copper directly during the carrying out of the necessary steps, and at the same time avoids the disadvantage of having to carry out a substantial number of steps in a wet way.

It will be further seen that there are many advantages in this invention. Some of the more improved ones may be appropriately indicated as giving a material improvement in the general economy of production of nickel and copper; giving greater economy in the production of copper by producing it in a readily saleable form as in blister form; giving improvements in some of the steps of the process, some of which steps

have heretofore been known in a general way; giving nickel substantially cobalt free, and producing it in the desirable form of pellets; and permitting the process to be carried out in the dry way, thereby eliminating costly handling charges. Also, it is to be particularly pointed out that both the nickel and copper are produced in their most desirable forms by the single continuous process.

10 When in the specification and claims I refer to carbon monoxide as the medium or agent for recovering nickel from metallic masses containing nickel and other metals, 15 I intend to include other substances which will be equivalent to and function the same as carbon monoxide.

What is claimed is:

1. The process of recovering commercially pure metallic nickel from nickel-copper ores or mattes in a dry way free from wet operations involving the dissolution of nickel and/or copper, which comprises smelting nickel-copper ores or mattes with material yielding an alkaline sulphide to convert said ore or matte and said material into a molten mass, permitting said molten mass to remain practically undisturbed whereby copper sulphide floats to the top of the mass and nickel sulphide contaminated with some copper sulphide settles to the bottom of the mass, removing said copper sulphide from the top of the mass, smelting said nickel sulphide with material capable of yielding an alkaline sulphide, maintaining said nickel sulphide mass in a molten state whereby copper sulphide floats to the top of the mass and nickel sulphide settles to the bottom, removing said copper sulphide tops and returning the same for use in the first smelting, comminuting the nickel sulphide bottoms, roasting said comminuted material to convert the same into an oxide, subjecting the oxide to heat in the presence of a reducing gas including water gas, treating the reduced mass containing metallic nickel with carbon monoxide to form gaseous nickel carbonyl, passing said gaseous nickel carbonyl over pellets of nickel under thermal conditions capable of decomposing said nickel carbonyl into commercially pure nickel substantially free from cobalt and carbon monoxide, and recovering the carbon monoxide for reuse in the treatment of further amounts of the aforesaid reduced metallic mass, all of the aforesaid operations being free from wet operations involving the dissolution of nickel and/or copper.

2. The process of recovering commercially pure metallic nickel as set forth in claim 1 in which material yielding sodium sulphide is used in the smelting of nickel-copper ores or mattes to convert the same into a molten mass in which copper sulphide separates to the top thereof and nickel sulphide settles to the bottom thereof.

3. The process of recovering commercially pure nickel from nickel-copper ores or mattes in a dry way free from wet operations involving the dissolution of nickel and/or copper which comprises concentrating nickel sulphide from nickel-copper ores or mattes by smelting with an alkaline sulphide to effect a separation of nickel sulphide from copper sulphide, roasting the concentrated nickel sulphide to oxidize nickel, reducing nickel oxide to metallic nickel by a gaseous reducing agent, volatilizing said metallic nickel as nickel carbonyl and decomposing said carbonyl to produce commercially pure nickel.

In testimony whereof, I have hereunto set my hand.

ROBERT C. STANLEY.

70

75

80

85

90

95

100

105

110

115

120

125

130